

## UNITED STATES PATENT OFFICE

HARRY S. GEORGE, OF MASSAPEQUA, NEW YORK, ASSIGNOR TO ELECTRO METALLURGICAL COMPANY, A CORPORATION OF WEST VIRGINIA

## FINISHED IRON-CHROMIUM ALLOY ARTICLE AND METHOD OF MAKING THE SAME

No Drawing. Application filed December 21, 1928, Serial No. 327,757. Renewed November 23, 1931.

My invention relates to finished articles consisting of iron-chromium alloys containing 8% to 40% chromium, and especially to rustless iron and stainless steel articles which contain less than .3% carbon and to methods 5 of producing the same.

Articles consisting of these iron-chromium alloys are shaped by hot rolling or forging methods. Heretofore, the articles have been 10 box annealed at 800° to 1000° C. to bring about structural changes in the alloy and to produce ductility. The rolled or forged articles are covered with an oxide scale and the annealing is done with the oxide present on 15 the surface of the metal. The surface oxide on these box annealed metals is extremely resistant to pickling acids and on some of the metals it is practically immune to the action of acid. The removal of the surface oxide on such annealed articles has required a prolonged treatment in an acid bath, a grinding 20 operation, or sand blasting. These cleaning methods remove a considerable amount of metal and destroy the surface finish and they are laborious and costly. It has not been 25 helpful to remove the oxide before the metal is box annealed because a similar acid resistant oxide is produced when clean metal is box annealed and the same destructive methods had to be used to clean it.

I have discovered new methods of treating 30 such alloys which avoid these difficulties and reduce the cost of production. The oxides which occur on these alloys after they are 35 hot rolled may be removed in acid pickling baths. I prefer to remove the oxides in a dilute acid bath consisting of a mixture of nitric and hydrochloric acids but other acids may be used. For example, the hot rolled 40 scale on a rustless iron containing 18% chromium may be removed in a bath consisting of 10 grams per liter hydrochloric acid and 50 grams per liter nitric acid at about 70° C. without attacking the metal. 45 This bath will not attack the metal and destroy the hot rolled finish but will readily loosen the scale so that it will fall off. A higher concentration of hydrochloric acid may be used for alloys containing a higher 50 content of chromium and more dilute acids

are suitable for alloys of lower chromium content. These acids cause the hot rolled scales to peel or slough off practically undissolved.

After the oxide is removed the article is 55 box annealed in an atmosphere which is preferably non-oxidizing or reducing and which at all events is not strongly oxidizing. A coating of oxide so heavy that the finish will be destroyed or the metal will be unevenly 60 or diversely oxidized is avoided. A reducing atmosphere may be produced by displacing the air which is initially entrapped in the box with any reducing gas which will not deposit carbon when heated to 800° to 1000° 65 C. in contact with the metal. Box annealing the metal in contact with carbon in any form is to be avoided as the carbon forms a coating on these iron-chromium alloys which is difficult to remove. I have used a small quantity of wood charcoal in the annealing box 70 out of contact with the metal to produce the desired atmosphere and carefully luted the box to prevent oxidizing gases from entering. For this purpose, I prefer to use lump wood charcoal. The charcoal combines with practically all of the oxygen entrapped in the box 75 and prevents the formation of more than an extremely thin film of oxide on the metal. The metal is heated to about 800° to 1000° 80 C. for a time sufficient to bring about ductility and structural changes according to the annealing practice which is well understood in the art.

The annealed article has a thin coating of 85 oxide which resembles the oxide surface known as temper color. For the purposes of this invention, this thin coating will be referred to herein as an iridescent coating.

The coating is so thin that the article can be 90 considered as finished at this stage but if desired a novel method of cleaning may be used to remove the iridescent coating. The iridescent coating is so resistant to acid that it cannot be removed in an acid bath without destroying the surface finish but it may be removed by means of the method of cleaning described in my co-pending application entitled Method of removing oxide coatings 95 from metals, Serial No. 327,756, filed Decem- 100

ber 21, 1928. In accordance with this method the article may be treated in a 15% to 30% sodium hydroxide solution to which chlorine has been added until the solution is 5 clouded with liberated oxygen. Merely dipping the article in this solution is usually sufficient but a longer treatment in the alkali solution is not harmful. The alkali changes the character of the scale so that acids will 10 remove it. I prefer to use an acid bath which will not materially attack the metal. Dipping the alkali treated article into a bath like the one used to remove the hot rolled scale will ordinarily remove the iridescent coating 15 in a few seconds without attacking the metal or materially changing the character of the surface given to it in hot working.

My invention provides a new annealed article of iron-chromium alloy with a finished 20 surface of an iridescent oxide, which is so thin that the utility of the article is not impaired for many purposes. An article with an oxide-free surface is provided by less costly methods than those heretofore used and 25 extremely small amounts of metal and pickling materials are consumed.

Since various modifications of the process may be made without departing from my invention, I do not wish to limit my invention 30 except by the prior art and by the invention as defined in the annexed claims.

I claim as my invention:

1. An annealed article consisting of an iron-chromium alloy containing 8% to 40% 35 chromium having a hot rolled finish and a thin iridescent oxide coating.
2. An annealed article consisting of an iron-chromium alloy containing 8% to 20% chromium having a hot rolled finish and a 40 thin iridescent oxide coating.
3. An annealed iron-chromium alloy containing 8% to 40% chromium and carbon not in excess of .3% and having an unpolished unetched hot rolled surface finish free 45 from surface oxides.

4. The method of producing a finished article of iron-chromium alloy containing 8% to 40% chromium which comprises treating the hot rolled article in an acid bath to 50 remove only the surface oxides and then box annealing in the presence of wood charcoal which is out of contact with the metal.

5. The method of producing a finished iron-chromium alloy article containing 8% 55 to 40% chromium which comprises treating the hot rolled article in an acid bath to remove only the surface oxides and then box annealing in a non-carburizing atmosphere which is not strongly oxidizing.

6. The method of producing a finished iron-chromium alloy article containing 8% to 40% chromium which comprises treating the hot rolled article in an acid bath to remove 60 only the surface oxides and then box annealing at 800° to 1000° C. in the presence

of solid carbon under such conditions that the carbon is out of contact with the article whereby to yield an atmosphere which is non-carburizing and not strongly oxidizing.

7. The method of producing a finished 70 iron-chromium article containing 8% to 40% chromium which comprises treating the hot rolled article in an acid bath to remove only the surface oxides, heating to 800° to 1000° C. in a closed container in the presence of 75 solid carbon under such conditions that the carbon is out of contact with the metal whereby to yield an atmosphere which is non-carburizing and not strongly oxidizing, immersing 80 in an alkali bath and then in an acid bath which will not attack the metal.

8. The method of producing a finished 85 iron-chromium article containing 8% to 40% chromium which comprises treating the hot rolled article in an acid bath to remove only 90 the surface oxides, heating to 800° to 1000° C. in a closed container in the presence of solid 95 carbon under such conditions that the carbon is out of contact with the metal whereby to yield an atmosphere which is non-carburizing and not strongly oxidizing, immersing 100 in an alkali bath containing an oxidizing agent and then in an acid bath.

9. The method of producing a finished 105 iron-chromium alloy article containing 8% to 40% chromium which comprises treating the hot rolled article in a bath at about 70° C. containing about 10 grams per liter hydrochloric acid and 50 grams per liter nitric acid, annealing in a closed container in the presence of solid carbon under such conditions that the carbon is out of contact with the metal, treating in a solution containing about 20% sodium hydroxide and a small 110 amount of chlorine and then in said acid bath.

10. The method of producing a finished 115 iron-chromium article containing 8% to 40% chromium which comprises treating the hot rolled article in an acid bath to remove surface oxides so that the surface finish will not be impaired, heating to 800° to 1000° C. in a closed container in the presence of wood charcoal under such conditions that the charcoal is out of contact with the metal, treating 120 in an alkali bath and then in an acid bath.

11. The method of producing a finished 125 iron-chromium article containing 8% to 40% chromium which comprises treating the hot rolled article in an acid bath so as to remove surface oxides without impairing the surface finish, annealing in a closed container in the presence of solid carbon under such conditions that the carbon is out of contact with the metal, treating in a bath containing about 20% sodium hydroxide to which chlorine has been added and then in an acid bath 130 containing about 10 grams per liter hydro-

chloric acid and 50 grams per liter nitric acid.

12. The method of producing a finished iron-chromium article containing 8% to 40% chromium which comprises treating the hot rolled article in an acid bath containing about 10 grams per liter hydrochloric acid and 50 grams per liter nitric acid, annealing in a closed container in the presence of wood charcoal under such conditions that the charcoal is not in contact with the metal, treating in a bath containing about 20% sodium hydroxide to which chlorine has been added and then in the said acid bath.

15 In testimony whereof I affix my signature.  
HARRY S. GEORGE.

20

25

30

35

40

45

50

55

60

65